

# UNITED STATES PATENT OFFICE.

WILLIAM A. McADAMS, OF BAY SHORE, NEW YORK.

## ALUMINUM ALLOY.

1,212,374.

Specification of Letters Patent. Patented Jan. 16, 1917.

No Drawing. Application filed April 15, 1914, Serial No. 332,053. Renewed June 6, 1916. Serial No. 102,089.

*To all whom it may concern:*

Be it known that I, WILLIAM A. McADAMS, a citizen of the United States, and resident of Bay Shore, in the county of Suffolk and State of New York, have invented a new and useful Improvement in Aluminum Alloys, of which the following is a specification.

My invention relates to an aluminum alloy with the object in view of providing a stiff and strong casting alloy particularly well suited for small castings.

With this end in view, my invention consists of an aluminum alloy composed of aluminum, zinc and copper, in which the proportion by weight of zinc exceeds the copper and the aluminum exceeds the zinc. The aforesaid elements are preferably combined in substantially the proportions by weight of one hundred eight parts aluminum, forty-six parts zinc and twenty parts copper.

In preparing the alloy, a portion of the aluminum is first melted and raised to a

heat sufficiently high to fuse the copper, the 25 copper is then introduced and after the mass is somewhat cooled, the zinc is introduced. During the introduction of the elements, the mass should be kept thoroughly agitated. When all the elements have been introduced, 30 the mass while still in a fluid state may be poured into ingots for shipment or for immediate use as a casting metal and will be found very stiff and strong.

What I claim is:

An aluminum alloy composed of aluminum, zinc and copper in substantially the proportion by weight of one hundred and eight parts aluminum, forty-six parts zinc and twenty parts copper.

In testimony, that I claim the foregoing as my invention, I have signed my name in presence of two witnesses, this 14th day of April, 1914.

WILLIAM A. McADAMS.

Witnesses:

F. GEORGE BARRY,  
LIDA M. EGBERT.